

3,166,412  
CAST NICKEL-BASE ALLOY FOR GAS  
TURBINE ROTORS

Clarence G. Bieber, Roselle Park, N.J., assignor to The International Nickel Company, Inc., New York, N.Y., a corporation of Delaware  
No Drawing. Filed Aug. 31, 1962, Ser. No. 220,857  
4 Claims. (Cl. 75—171)

The present invention relates to alloys suitable for use under stress over a wide range of temperatures and, more particularly, to cast nickel-base alloys which are particularly suitable for the production of gas turbine rotors having the blades cast integrally with the hub.

It is well known that various nickel-base alloys employed in either the cast or wrought form are very useful for the production of blades which must operate at very high temperatures such as 1700° F., 1800° F., and higher in gas turbines employed in aircraft and in other applications. Generally, for aircraft applications, the nickel-base alloy blades are produced individually and are then fastened into a rotor hub which is made of a different alloy to produce a composite turbine rotor. Since the hub portion of the rotor is not required to operate at the very high temperatures to which the blade portions of the rotor are subjected, the metal or alloy which is employed for the rotor hub is required only to have good strength and ductility over the temperature range from approximately room temperature up to possibly 1000° F. or 1200° F. In the production of turbine rotors for use in gas turbines of relatively small size which can be employed in automotive gas turbine applications, the economic picture is quite different from that which exists in the case of aircraft gas turbines. Thus, it is no longer economically feasible to produce the blades separately and then fasten them to the rotor hub so as to form a composite turbine rotor. It has accordingly been proposed to produce the turbine rotor as a unitary casting having the blades integrally cast into the hub. Since the blade portions of the rotor are subjected to completely different combinations of stress and temperature than is the hub portion of the rotor, a vexing metallurgical problem is created since it is necessary to provide within a single unitary casting metallurgical structures which will operate under vastly different conditions of stress and temperature. It is known that alloys which are satisfactory for service in the rotor hub are unsatisfactory as blade materials. On the other hand, it has been found in practice that the alloys which are satisfactory as the blade materials are not satisfactory for use in the hub portion of the rotor. Accordingly, a demand has arisen for a nickel-base casting alloy having properties which would render it at the same time satisfactory for use as a cast rotor hub material and for use as a cast turbine blade material.

Although attempts have been made to overcome the foregoing difficulties and other difficulties, none, as far as I am aware, was entirely successful when carried into practice commercially on an industrial scale.

It has now been discovered that particular cast nickel-base alloys having special contents of chromium, aluminum, titanium, columbium, molybdenum, and carbon are particularly useful for the production of unitary gas turbine rotors having the blades cast integrally with the hub.

It is an object of the present invention to provide a cast alloy capable of withstanding high stress at elevated temperature for relatively long periods of time.

Another object of the present invention is to provide a cast alloy having high combinations of strength and ductility at usual ambient temperatures.

The invention also contemplates providing gas turbine

rotors made of the special cast alloy provided in accordance with the invention and which have the blades cast integrally with the hub.

Other objects and advantages will become apparent from the following description.

Generally speaking, the present invention provides cast nickel alloys containing, in percent by weight, not more than about 0.05% or 0.06% carbon, e.g., about 0.03% carbon, about 10% to about 18% chromium, about 5% to about 7% aluminum, up to about 1.5% titanium, e.g., 0.5% to about 1.5% titanium, about 1% to about 3% columbium, about 0.5% to about 6% molybdenum, with the chromium plus molybdenum contents being about 15% to about 20% of the alloy, up to about 0.05% boron, up to about 0.15% zirconium, up to about 0.05% calcium, and the balance essentially nickel. For best combinations of strength and ductility, chromium advantageously is maintained in the range of 10% to 14%. The total content of chromium and molybdenum in the alloy is important and must be maintained in the range of 15% to 20% in order to provide the best combination of corrosion resistance, strength, and ductility at elevated temperatures. Aluminum is an important hardening and strengthening element in the alloy and is maintained in the range of 5% to 7% because strength is sacrificed if the concentration of this element is too low while the ductility is lowered if the concentration is above 7%. Titanium, when present even in amounts of about 0.5%, contributes further hardening and strengthening to the alloy but should not exceed about 1.5% of the alloy because ductility and castability are reduced if the titanium content is higher than this value. Columbium also plays an important part in strengthening the alloy and is employed in amounts of 1% to 3% because strength is sacrificed if the concentration of this element is below 1% while the ductility is reduced if the concentration is above 3%. Boron and zirconium present in the alloy contribute markedly to the development of satisfactory strength and ductility properties therein. Thus, the presence of as little as 0.005% boron and at least about 0.02% zirconium provide good ductility at temperatures above about 1000° to 1200° F. Calcium in the alloy is employed in air melting to serve as a deoxidizer. It is omitted in vacuum melting. It is to be understood that carbon in the alloy must be maintained at very low values not exceeding 0.06% in order that the alloys will exhibit the required high elongation in the as-cast condition at room temperature even in sections as heavy as three inches thick or more. Small carbon contents of about 0.03% are beneficial in producing the master alloy which is to be remelted to make the finished castings. The alloy provided in accordance with the invention may also contain up to 15% cobalt, e.g., about 10% cobalt, as such amounts of cobalt permit the inclusion in the alloy of as much as about 8% of aluminum without encountering serious embrittling effects. Tungsten may be employed in place of a part or all of the molybdenum in the alloy. The alloy should be as devoid as practicable of impurities such as sulfur, phosphorus, lead, antimony, tin, selenium, tellurium, bismuth, etc. Elements such as silicon and manganese are undesirable and should not be present in amounts exceeding about 0.2% and 0.1%, respectively. Iron is also an undesirable element in the alloy and should not be present in amounts exceeding about 0.5%, e.g., about 0.25%. The balance of the alloy is essentially nickel.

The alloy provided in accordance with the invention is characterized by a room temperature tensile strength in the as-cast condition of at least about 100,000 p.s.i. and an elongation of at least about 10% in the as-cast condition. In addition, the alloy provides relatively long service life at temperatures on the order of about 1700° F. to

1800° F. For example, the alloy will usually provide a rupture life of at least about 22 hours when tested at 1800° F. and 22,000 p.s.i. and will usually have a service life of at least about 50 hours when tested at 1700° F. and 30,000 p.s.i. in the as-cast condition.

The following tables contain, respectively, the chemical compositions, in percent by weight, of vacuum melted and vacuum cast alloys produced in accordance with the invention, the rupture lives of the alloys at 1700° F. and 30,000 p.s.i. in the as-cast condition, and the room temperature tensile properties of these alloys in the as-cast condition:

Table I

| Alloy No. | Percent Cr | Percent Mo | Percent Cb | Percent Al | Percent Ti | Percent C | Percent B | Percent Zr | Percent Ni |
|-----------|------------|------------|------------|------------|------------|-----------|-----------|------------|------------|
| 1         | 12         | 5          | 2          | 6          | 0.6        | 0.008     | 0.01      | 0.10       | Bal.       |
| 2         | 12         | 5          | 2          | 6          | 0.6        | 0.05      | 0.01      | 0.10       | Bal.       |

Table II

| Alloy No. | Rupture Life, Hours, 1700° F., 30,000 p.s.i. | Percent Elongation |
|-----------|----------------------------------------------|--------------------|
| 1         | 57.2                                         | 12.4               |
| 2         | 74.0                                         | 24                 |

Table III

| Alloy No. | Yield Strength, p.s.i. | Ultimate Tensile Strength, p.s.i. | Percent Elongation |
|-----------|------------------------|-----------------------------------|--------------------|
| 1         | 95,000                 | 118,000                           | 29                 |
| 2         | 102,000                | 131,000                           | 14                 |

In contrast to the properties developed in the foregoing alloys, another alloy identical in composition to Alloy No. 2 set forth hereinbefore except that it contained 0.12% carbon was found to have a satisfactory rupture life of 64 hours at 1700° F. and 30,000 p.s.i. together with a room temperature yield strength of 104,000 p.s.i. and a room temperature tensile strength of 126,000 p.s.i. but was found to have an elongation at room temperature of only 6%.

Alloys in accordance with the invention have particularly satisfactory properties when produced by vacuum melting. They may, however, be melted under argon or even under air atmospheres with good castability and with only slight sacrifice in properties as compared to those produced by vacuum melting.

The strength of the alloy at room temperature and at elevated temperatures may be improved by subjecting the castings to a heat treatment comprising a heating at about 2150° F. for about 15 minutes to about 24 hours, e.g., about two hours, followed by a cooling to room temperature. If desired, a further stabilization treatment consisting of a heating at about 1700° F. for about one to about 24 hours, e.g., about four hours, may also be employed. In casting the alloy, it is important to superheat the melt to a temperature of at least 300° F., but more advantageously at least about 400° F. or 500° F., e.g., 600° F., about the freezing temperature thereof. For example, a pouring temperature of about 2950° F. is very satisfactory.

The alloy provided in accordance with the present in-

vention is particularly applicable to the production of castings, such as turbine rotors having the blades integrally cast with the hub, which have at least one included section subjected in use to high stress at temperatures on the order of about 1700° F. and have at least one included section subjected in use to high stress at temperatures on the order of about 1000° F. Such castings produced in accordance with the invention provide satisfactory properties although portions thereof are subjected to very different service temperatures from those to which other portions of the casting are subjected. The castings have improved fatigue strength.

As will be readily understood by those skilled in the art, the expression "balance essentially nickel" does not exclude the presence of other elements commonly present in such alloys as incidental elements, e.g., deoxidizing and cleansing elements, and impurities ordinarily associated therewith in small amounts which do not adversely affect the basic characteristics of my alloys.

20 Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and appended claims.

I claim:

1. A casting having at least one included section subjected in use to high stress at temperatures on the order of about 1700° F. and at least one included section subjected in use to high stress at temperatures on the order of about 1000° F., made of an alloy consisting essentially of about 0.008% to 0.05% carbon, about 12% chromium, about 5% molybdenum, about 6% aluminum, about 0.6% titanium, about 2% columbium, about 0.01% boron, about 0.1% zirconium, and the balance essentially nickel.

40 2. A nickel-base alloy containing not more than about 0.06% carbon, about 10% to 18% chromium, about 0.5% to 6% of a metal from the group consisting of molybdenum and tungsten and with the total contents of chromium, molybdenum and tungsten being about 15% to about 20%, about 5% to 8% aluminum, up to about 15% cobalt with the proviso that when the cobalt content is less than about 10% the aluminum content is about 5% to 7%, up to about 1.5% titanium, about 1% to 3% columbium, about 0.01% boron, up to about 0.15% zirconium, up to about 0.05% calcium, and the balance essentially nickel.

45 3. A nickel-base alloy according to claim 1 wherein the chromium content is about 10% to about 14%.

50 4. A nickel-base alloy consisting essentially of about 0.05% carbon, about 12% chromium, about 5% molybdenum, about 6% aluminum, about 0.6% titanium, about 2% columbium, about 0.01% boron, about 0.1% zirconium, and the balance essentially nickel.

## References Cited in the file of this patent

## UNITED STATES PATENTS

- 2,912,323 Bieber et al. ----- Nov. 10, 1959  
 2,975,051 Wilson et al. ----- Mar. 14, 1961  
 3,005,704 Faulkner ----- Oct. 24, 1961

## FOREIGN PATENTS

- 548,777 Canada ----- Nov. 12, 1957  
 733,489 Great Britain ----- July 3, 1955

UNITED STATES PATENT OFFICE  
CERTIFICATE OF CORRECTION

Patent No. 3,166,412

January 19, 1965

Clarence G. Bieber

It is hereby certified that error appears in the above numbered patent requiring correction and that the said Letters Patent should read as corrected below.

Column 3, line 65, for "about" read -- above --.

Signed and sealed this 6th day of July 1965.

(SEAL)

Attest:

ERNEST W. SWIDER  
Attesting Officer

EDWARD J. BRENNER  
Commissioner of Patents